

# UNITED STATES PATENT OFFICE.

HENRY PANNILL, OF PETERSBURG, VIRGINIA.

## PROCESS OF MAKING MOVING-PICTURE SCREENS.

1,149,940.

Specification of Letters Patent. Patented Aug. 10, 1915.

No Drawing.

Application filed December 16, 1913. Serial No. 807,134.

To all whom it may concern:

Be it known that I, HENRY PANNILL, a citizen of the United States, residing at Petersburg, in the county of Dinwiddie and State of Virginia, have invented new and useful Improvements in Processes of Making Moving-Picture Screens, of which the following is a specification.

This invention relates to process of producing moving picture screens.

The object of the invention is to produce an improved type of screen which will have substantially the same effect of a mirror screen and may be produced at one-fifth of the cost.

Another object of the invention is the provision of a screen which will not affect the eyes when pictures are viewed thereon at short distances and which will have the effect of throwing the pictures in relief.

Further objects of the invention will appear as the following description is read.

In carrying out the present invention I apply to one side of a canvas of the proper size a composition of equal quantities of linseed oil and Japan drier. This coating is allowed to stand for twelve hours when the canvas is turned over and a coating applied to the opposite side consisting of a mixture of three parts water and one part alcohol. This last coating removes the stiffening, or, in other words, takes the life out of the canvas and makes it supple and prevents the same from cracking. A mixture of one part dry aluminum and three parts bronze liquid is then applied to the side first coated and after twelve hours' drying time has elapsed a coating of dry aluminum powder or gold powder is applied and rubbed in thoroughly with a brush after which a bright polish may be produced by rubbing the surface with Turkish toweling or like material.

If it is found that the canvas is spotted after the first application of aluminum and

bronze liquid, a mixture of three parts shellac varnish and one part alcohol should be applied. After approximately twelve hours have elapsed a second coating of aluminum and bronze liquid (one part aluminum and three parts bronze liquid) should be applied. This should be allowed to dry at least one hour and then covered with a dry aluminum powder and rubbed in with a brush. After this the surface may be polished as before. This will produce a screen having a bright mirror-like surface which is of sufficient roughness to properly reflect the rays of light impinging against the same and which is thoroughly pliable and supple.

What is claimed is:

1. The process of producing moving picture screens which consists in coating one side of the canvas with a sizing, and subsequently coating the opposite side with a liquid adapted to take the life out of the canvas and to render it supple, coating the side first coated with a substance arranged to produce a bright surface and finally rubbing an aluminum or gold powder into the surface first coated and polishing the same.

2. The process of producing moving picture screens which consists in applying to one side of a canvas the composition of equal parts of linseed oil and Japan drier, subsequently applying to the opposite side a mixture of three parts of water and one part alcohol, then applying a mixture of one part dry aluminum powder and three parts bronze liquid to the side first coated and finally rubbing into the side first coated an aluminum or gold powder and polishing the same.

In testimony whereof I affix my signature in presence of two witnesses.

HENRY PANNILL.

Witnesses:

PAUL PETTIT,

CHARLES E. POLLARD.